

Oct. 3, 1967

R. E. ORMSBEE

3,344,741

RECEIVING SHEET FOR USE AS A MASTER OR COPY IN THE DTR PROCESS

Filed Sept. 20, 1965



FIG. 1



FIG. 2



FIG. 3

INVENTOR  
Ruth E. Ormsbee

by McDougall, Hersh & Scott  
Attn:ys

## 1

3,344,741

 RECEIVING SHEET FOR USE AS A MASTER OR  
COPY IN THE DTR PROCESS

Ruth E. Ormsbee, River Forest, Ill., assignor to A. B. Dick Company, Niles, Ill., a corporation of Illinois  
Filed Sept. 20, 1965, Ser. No. 488,479  
4 Claims. (Cl. 101—462)

This invention relates to the production of copy by the diffusion transfer reversal process, generally referred to as the DTR process, and it relates more particularly to the preparation of an image receiving sheet which can be used both as a sheet for the production of single copies or as a master from which multiple copies can be produced by lithographic duplication. More specifically, the invention relates to a lithographic master which can be imaged by the DTR process and which can also be used as a single copy sheet.

Copy sheets for use in the production of single copy by the DTR process have been available for some time; however, such sheets cannot generally be employed as lithographic masters from which multiple copies of good quality can be produced when imaged by DTR technique.

The difficulty in the fabrication of a lithographic master for imaging by diffusion transfer resides in the formulation of a sheet which embodies the characteristics essential for lithographic reproduction, including (1) a sheet having high wet strength and dimensional stability to enable repeated wetting with aqueous repellent and oleophilic ink composition in the production of inked copies therefrom, (2) which embodies a water insoluble, water receptive, ink repellent surface essential to the imaged master, and (3) which has surface characteristics that provide the critical balance between water receptivity in the non-imaged portions and ink receptivity in the imaged portions whereby the aqueous repellent with which the sheet is first wet will preferentially be received by the non-imaged hydrophilic portions of the imaged master while the precipitated silver image deposited on the surface diffusion transfer from an exposed negative will repel the aqueous repellent and be preferentially wet by the oleophilic ink composition in inking the master for use in the production of copy.

To the present, it has only been possible to make use of a DTR lithographic plate formed of an aluminum base sheet having a surface treated to render the surface hydrophilic and lithographic as by reaction with a water soluble silicate, acrylic acid, or by anodization to form an oxide layer and in which the lithographic surface is provided with a nucleating agent, such as colloidal silver, silver sulfide, cadmium sulfide and the like for nucleating the conversion of the soluble silver halide complex diffused from the unexposed portions of the negative to precipitate silver as an ink receptive, water repellent image on the lithographic surface of the aluminum sheet.

Such aluminum lithographic plates are, of course, expensive and unsuitable for use as single copy whereby the plate is limited to applications where an extremely large number of copies are to be produced.

DTR plates for lithographic duplication have been formed of coated paper base sheets wherein the paper base sheet is formulated to contain a resinous binder to impart wet strength and which is overcoated with a gelatin coating containing the nucleating agent. Such wet strength papers are non-lithographic such that the procedure required for preparation of the plate for lithographic duplication has included treatment of the surface of the plate, after the plate has been imaged, with an acid etch composition for conversion of the non-imaged portion of the plate to a hydrophilic, ink repellent, lithographic surface. Such multiple steps for the preparation of an

## 2

imaged master for lithographic duplication is objectionable, at least from the standpoint of time, labor and materials, and even then a satisfactory plate for the production of a large number of copies of good quality is difficult to achieve.

Further, the nucleating agent is incorporated in a gelatin coating applied to the surface of a paper base sheet. Gelatin coatings of the type described are difficult to apply and they also provide a surface which presents problems during image development by diffusion transfer in that the gelatin coating is adhesive and makes separation of the negative and positive sheets more difficult and it also retards drying and introduces curl into the master thereby to militate against the production of an imaged plate which lies flat on the plate cylinder of the duplicating machine.

It is an object of this invention to produce and to provide a method for producing a coated paper lithographic plate adapted for imaging from an exposed negative in a DTR process; which can be used interchangeably as a direct single copy or which can be used as an imaged lithographic master from which multiple inked copies can be produced by lithographic duplication; which does not require a pre-etch or etch applied after an image has been formed on the plate for rendering the non-imaged portions hydrophilic and lithographic; which provides the desired critical balance between the ink receptivity of the imaged portion formed on the plate and the water receptivity of the non-imaged portion; which does not require the use of a gelatin top coat for support of nucleating agent; which dries rapidly upon separation from the exposed negative to produce a flat, flexible, imaged master which can be mounted on the plate cylinder of a lithographic press; and from which a large number of copies of good quality can be produced.

These and other objects and advantages of this invention will hereinafter appear and for purposes of illustration, but not of limitation, an embodiment of the invention is shown in the accompanying drawing, in which

FIG. 1 is a perspective view partially in section of a receiving sheet embodying the features of this invention;

FIG. 2 is a sectional elevational view of the arrangement of elements for imaging the receiving sheet by an exposed negative; and

FIG. 3 is a perspective view partially in section similar to that of FIG. 1 showing the imaged receiving sheet.

The concepts of this invention will hereinafter be described by reference to a specific example for the preparation of a coated paper receiving sheet or master and the method for use of same in the preparation of an imaged lithographic plate from which multiple copies can be produced or which can be used as a single copy.

## Example 1

## Receiving sheet-coating composition:

|                                                                                |    |     |
|--------------------------------------------------------------------------------|----|-----|
| Water                                                                          | ml | 20  |
| Colloidal silica (30% SiO <sub>2</sub> )                                       | ml | 30  |
| Sodium sulfide (0.5% solution)                                                 | ml | 2.2 |
| Silver nitrate (0.5% solution)                                                 | ml | 3.0 |
| Polyvinylidene chloride latex (60% solids—<br>Serfene H30—Morton Chemical Co.) | ml | 1.5 |
| Acrylic emulsion polymer (46% solids—Rho-<br>plex AC33—Rohm & Hass Co.)        | g  | .25 |
| Saponin (10% solution)                                                         | ml | .01 |

The coating composition is applied by roller coating, flow coating or other suitable paper coating process in coating weights of 0.5 to 10.0 pounds per 3000 square feet of surface area, or to a water resistant paper base sheet such as Schoeller water resistant base, or Baryta paper and the like. The coating 12 is air dried or preferably

force dried in an air drying oven at a temperature within the range of 150-300° F.

After sheeting and punching to provide the openings 14 in the leading edge of the sheet for mounting as a lithographic plate onto a plate cylinder of a lithographic press, the coated paper is ready for use as a receiving sheet.

#### Example 2

**Imaging.**—For imaging by DTR process, use is made of a negative sheet 20 of the type presently employed in single copy work or a type of negative preferably employed with the commercial aluminum plates imaged by the DTR process. Such negative sheets, embodying a silver halide-gelatin coating 22 on a suitable plastic film 24 or paper base sheet, are marketed by Agfa-Gevaert, Inc., Peerless Photo Products, Inc. and by Anken Chemical and Film Corporation, the latter being referred to as the Anken contact negative.

After exposure of the negative to the original or other subject matter to be reproduced, the exposed negative is brought into surface contact with the coated side of the receiving sheet after the exposed negative or both the negative and the receiving sheet have been wet with a conventional developing solution, as represented by the following developing composition, which is diluted in the ratio of 1 to 1 with tap water before use.

#### Example 3

Developer composition:

|                            |        |       |    |
|----------------------------|--------|-------|----|
| H <sub>2</sub> O           | ml.    | 800   | 30 |
| Phenidone                  | g.     | 3.0   |    |
| Sodium sulfite             | g.     | 163.0 |    |
| Hydroquinone               | g.     | 30.0  |    |
| Sodium hydroxide           | g.     | 30.0  |    |
| Sodium thiosulfate-penta   | g.     | 20.0  |    |
| Potassium bromide          | g.     | 3.0   |    |
| H <sub>2</sub> O to volume | quart. | 1     |    |

In response to wetting with the developing solution, the exposed portion 26 of the silver halide coating is reduced to silver while the silver halide in the relatively unexposed portion 28 is converted into a soluble silver halide complex which dissolves in the solution for transfer by diffusion from the exposed negative to the coated surface of the receiving sheet.

The nucleating agent present in the surface of the receiving sheet operates to reduce the silver halide complex to colloidal particles of silver or other reduction reaction product which becomes strongly bonded to the coated surface of the sheet and defines an oleophilic, ink receptive, water repellent image 30 on an otherwise ink repellent, water receptive hydrophilic, water insoluble, lithographic surface.

The receiving sheet is then separated from the negative sheet. Separation is easy by reason of the absence of gelatin in the coating 12 on the receiving sheet and also by reason of the presence of colloidal silica as an essential and major component of said coating. The separated receiving sheet also appears immediately to dry possibly because of the presence in the coating of colloidal silica. In any event, the imaged sheet can be used directly as a single copy or it can be immediately, or after a period of time, mounted on the plate cylinder of a lithographic press for use in the production of a number of inked copies by conventional lithographic duplicating technique. However, it is preferred to fix the image and condition the plate by treatment of the imaged surface with a conditioner represented by the following:

#### Example 4

Conditioner:

|                                                                  |     |      |
|------------------------------------------------------------------|-----|------|
| H <sub>2</sub> O                                                 | ml. | 69.5 |
| Carboxymethylhydroxyethyl cellulose-43 low (Hercules Powder Co.) | g.  | 0.2  |
| Sodium nitrate                                                   | g.  | 2.0  |
| Ammonium phosphate                                               | g.  | 1.0  |

|                         |    |      |
|-------------------------|----|------|
| Glycerine               | g. | 19.0 |
| Ethyl alcohol           | g. | 7.0  |
| Cetylpyridinium bromide | g. | 0.05 |

5 The conditioner is wiped onto the surface of the image receiving sheet, before or after mounting on the press, and then inked copies are produced by first wetting the surface with aqueous repellent to wet out the unsilvered, non-imaged portions 32 of the plate and then wetting with 10 an oleaginous ink composition which is not received by the wet non-imaged portions but is received by the unmet oleophilic portions 30 for transfer of the ink image from the sheet to copy paper in a direct lithographic process or to a blanket in an offset process of lithographic duplication.

15 It will be understood that the formulation of the developing solution and the conditioner is not critical to the invention in that conventional photographic developers and lithographic conditioners can be employed.

20 An important concept of this invention resides in the non-gelatin coating applied to the paper base sheet for use in the preparation of the receiving sheet. It is not essential for the polyvinylidene chloride and the acrylic emulsion polymer to be present in the coating composition or for both to be present together in combination with the colloidal silica since either one or the other can be employed or the colloidal silica can be employed alone, as illustrated by the following examples:

#### Example 5

|                                                           |     |    |
|-----------------------------------------------------------|-----|----|
| Water                                                     | ml. | 30 |
| Colloidal silica (30% SiO <sub>2</sub> —Ludox LS—Du Pont) | ml. | 30 |
| Sodium sulfide (0.5% solution)                            | ml. | 2  |
| Silver nitrate (0.5% solution)                            | ml. | 3  |
| Polyvinylidene chloride latex (60% solids)                | ml. | 4  |
| Saponin (10% solution)                                    | ml. | 4  |

#### Example 6

|                                                           |     |    |
|-----------------------------------------------------------|-----|----|
| Water                                                     | ml. | 15 |
| Colloidal silica (30% SiO <sub>2</sub> —Ludox HS—Du Pont) | ml. | 30 |
| Sodium sulfide (0.5% solution)                            | ml. | 2  |
| Silver nitrate (0.5% solution)                            | ml. | 3  |
| Acrylic emulsion polymer (46% solids)                     | ml. | .5 |
| Saponin (10% solution)                                    | ml. | .1 |

#### Example 7

|                                     |    |     |
|-------------------------------------|----|-----|
| Colloidal silica (Ludox LS—Du Pont) | g. | 100 |
| Silver sulfide (.34% solution)      | g. | 25  |
| Silver nitrate (.68% solution)      | g. | 25  |

55 The amount and type of nucleating agent can be varied depending upon the formulation of the developer and the composition of the silver halide negative although any conventional nucleating agents can be employed. In the use of sodium sulfide and silver nitrate, in the preferred practice of this invention, it is preferred to make use of the materials in the ratio of about 1 part by weight of sodium sulfide to 1-1.5 parts by weight of silver nitrate 60 although it is permissible to make use of the materials within the range which comprises 1 part by weight of the sodium sulfide to 0-2 parts by weight of silver nitrate.

When used, the amount of resinous solids in the coating composition, when based upon the SiO<sub>2</sub> content of 65 colloidal silica, can range from 9 parts by weight of SiO<sub>2</sub> to .25-5.0 parts by weight of the combined resinous polymers and 9 parts by weight of SiO<sub>2</sub> to 1-4 parts by weight of the resinous material when formed of acrylic emulsion polymer, or 9 parts by weight of SiO<sub>2</sub> to 0.5-5.0 parts by 70 weight of resinous binder when formed of polyvinylidene chloride, all on a solids basis. The amount of nucleating agent can be varied over a fairly wide range depending upon the agent employed but it is preferred to make use of an amount within the range of .1-.5 part by weight nucleating agent per 9 parts by weight of SiO<sub>2</sub>.

The saponin is a surface active agent derived from plant glucosides such as triterpenoid saponin but the surface active agent is not essential to the formulation of the coating composition since it serves primarily for the stabilization thereof and other surface active agents can be used.

It will be apparent from the foregoing that I have provided a new and improved receiving sheet for imaging by diffusion transfer reversal technique and in which the receiving sheet may be used as a single direct copy or as a lithographic master from which multiple copies of good quality can be produced.

It will be understood that changes may be made in the details of construction, formulation and operation without departing from the spirit of the invention, especially as defined in the following claims.

I claim:

1. A receiving sheet for imaging by a diffusion transfer reversal process comprising a paper base sheet and a coating on the surface of the paper base sheet consisting essentially of the combination of colloidal silica, a nucleating agent for reduction of a soluble silver halide complex to an oleophilic ink receptive imaging material and present in an amount within the range of 0.1 to 0.5 part by weight per 9 parts by weight of colloidal silica and in which the nucleating agent comprises the combination of sodium sulfide and silver nitrate present in the ratio of 1 part by weight of sodium sulfide to 1 to 1.5 parts by weight of silver nitrate, and a resinous binder selected from the group consisting of a vinylidene chloride polymer and an acrylate polymer and in which the coating is a water insoluble coating which is water receptive, ink repellent, hydrophilic and lithographic.

2. A receiving sheet as claimed in claim 1 in which the vinylidene chloride polymer is present in the coating

in an amount within the range of 0.5 to 5.0 parts by weight to 9 parts by weight of colloidal silica calculated as  $\text{SiO}_2$ .

3. A lithographic imaged master as claimed in claim 1 in which the resinous binder is an acrylate emulsion polymer present in an amount within the range of 0.1 to 4 parts by weight per 9 parts by weight of colloidal silica.

4. A receiving sheet for imaging by diffusion transfer reversal process comprising a paper base sheet and a coating on the surface of the paper base sheet consisting essentially of the combination of colloidal silica and a nucleating agent for reduction of soluble silver halide complex to an oleophilic ink receptive imaging material in which the nucleating agent is present in an amount within the range of 0.1 to 0.5 part by weight per 9 parts by weight of colloidal silica and in which the nucleating agent comprises the combination of sodium sulfide and silver nitrate present in the ratio of 1 part by weight of sodium sulfide to 1 to 1.5 parts by weight of silver nitrate and in which the coating is water insoluble, water receptive, ink repellent, hydrophilic and lithographic.

#### References Cited

##### UNITED STATES PATENTS

|    |           |         |               |       |           |
|----|-----------|---------|---------------|-------|-----------|
| 25 | 2,698,237 | 12/1954 | Land          | ----- | 96—29     |
|    | 3,062,648 | 11/1962 | Crawford      | ----- | 96—33     |
|    | 3,157,117 | 11/1964 | Relph et al.  | ----- | 101—149.2 |
|    | 3,161,508 | 12/1964 | Hepher et al. | ----- | 96—33     |
| 30 | 3,220,837 | 11/1965 | Land et al.   | ----- | 96—33     |
|    | 3,247,793 | 4/1966  | Beatty et al. | ----- | 101—149.2 |

ROBERT E. PULFREY, *Primary Examiner.*

J. A. BELL, *Assistant Examiner.*